

June 19, 1945.

E. E. HABIB ET AL

2,378,701

MANUFACTURE OF ARTICLES FROM LIQUID DISPERSIONS

Filed Nov. 16, 1943



FIG. 1



FIG. 2



FIG. 3



FIG. 4

FIG. 5



EMILE E. HABIB  
GORDON E. GOT  
Inventors

By Theodore C. Browne  
Attorney

## UNITED STATES PATENT OFFICE

2,378,701

MANUFACTURE OF ARTICLES FROM LIQUID  
DISPERSIONS

Emile E. Habib and Gordon E. Gott, Arlington,  
Mass., assignors to Dewey and Almy Chemical  
Company, North Cambridge, Mass., a corpora-  
tion of Massachusetts

Application November 16, 1943, Serial No. 510,444

3 Claims. (Cl. 18—53)

The present invention relates to the manufacture of hollow rubber objects and more particularly to the manufacture of large-size meteorological and radiosonde balloons by a coagulant dipping process.

Balloons of this type had been made until the recent past by a casting procedure. This was a slow process and gave control difficulties because of the sensitivity and lack of stability of the dispersion. These difficulties were avoided by the introduction of a coagulant dipping process in which the deposited layer of rubber is stripped from the dipping mold while it is still plastic and is subsequently inflated to the desired larger size. This process is described in detail in our copending application Serial No. 510,442, filed on the same day as the present application.

This improved dipping type process was found to be applicable to natural latex dispersions only with the limitation that the dipping compound be used before the percentage of sulfur combined on the rubber hydrocarbon had risen to more than 0.45%, based on the dry weight of the hydrocarbon. If a natural latex dispersion in which the combined sulfur on the rubber hydrocarbon exceeds 0.45% is used, the freshly deposited gels can not be stretched enough to get them off the mold without tearing them. If they are allowed to dry and thus acquire sufficient strength for stripping, then they can not be permanently enlarged enough by inflation because the material is no longer capable of sufficient plastic flow. This characteristic of the process means that the dipping bath must be freshly prepared and used when not more than a few days old. For laboratory scale operation, this characteristic is not a serious handicap, but those skilled in the art will appreciate immediately the difficulties it causes when the process is used on a factory scale.

It is the principal object of the present invention to overcome the difficulty described above; to provide a modification of the coagulant dipping process referred to above which will adapt it to efficient and economic factory scale operation; and to provide a means of preventing the combined sulfur of the dipping bath from rising to an undesirable amount before the bath is used.

We have discovered a satisfactory procedure for introducing a sufficiently large amount of a vulcanization accelerator into the wet gels formed in the process described in the application referred to above which will distribute the accelerator uniformly in the gel without local concentrations which would produce non-uniform cure. This procedure is availed of to accomplish the objects of the invention by omitting

from the dipping compound the accelerator, using the compound for dipping in the normal manner, and then introducing an accelerator into the formed objects. As a consequence of the absence of an accelerator from the compound, modern high-speed accelerators may be used with the process and the compounds do not materially change in their combined sulfur content upon ageing and, therefore, need not be freshly prepared.

The invention will be more fully understood from a reference to the accompanying drawing, in which

Figure 1 is an elevation partly in section of the dipping mold after it has been withdrawn from the dispersion with the deposited gel layer on its outer surface;

Figure 2 illustrates the step of introducing a vulcanization accelerator into the gel layer while it is still on the mold;

Figure 3 shows the step of stripping the formed object from the mold;

Figure 4 shows the object undergoing inflation, and

Figure 5 shows in elevation the dried object.

In practicing the process of the present invention, we make up a dipping compound from a dispersion of natural latex and also make up a suitable coagulant compound. The following example illustrates compounds which are suitable:

|                                                                 | Parts by weight<br>of solids |
|-----------------------------------------------------------------|------------------------------|
| Rubber latex (60% solids)                                       | 100.00                       |
| Potassium hydroxide <sup>1</sup>                                | 1.75                         |
| Zinc stearate                                                   | 1.00                         |
| Symmetrical di-beta-naphthyl para phenylene diamine             | 1.00                         |
| Formaldehyde condensation product of naphthalene sulphonic acid | 0.24                         |
| Titanium dioxide                                                | 1.00                         |
| Sulphur                                                         | 1.10                         |
|                                                                 | <hr/> 106.09                 |

<sup>1</sup>The amount will vary with different latices; sufficient should be used to give the dispersion a viscosity suitable for dipping.

The coagulant has the following composition:

|                               |             |
|-------------------------------|-------------|
| Bentonite                     | 150         |
| Water                         | 900         |
| Acetone                       | 1,321       |
| Calcium nitrate tetra hydrate | 1,250       |
| Glycerine                     | 55          |
| Glacial acetic acid           | 37          |
|                               | <hr/> 3,713 |

55 The ingredients are added in the order stated.

A suitably shaped balloon mold 1 is dipped into the coagulant composition and then withdrawn, forming on its surface a layer of coagulant 3. The coagulant-coated mold is then dipped into a bath of a dipping compound having the above composition and allowed to dwell therein for the time required to build up a deposited gel layer of the desired thickness on its outer surface. The mold 1 together with the deposited gel layer 5 on its surface is then immersed in a bath as shown in Figure 2 containing a suitable accelerator of vulcanization. The accelerator may be in solution or in suspension. For gels formed from the composition of Example 1, a suitable bath may be made by dissolving 10 parts of potassium pentamethylene dithiocarbamate in 90 parts of water, and the mold should be held in the accelerator for about 20 minutes. The mold is then withdrawn from the accelerator and the gel layer 5 is stripped from its surface by stretching the neck of the gel and sliding it downwardly off the form as shown in Figure 3. The gel layer is then placed on an inflating nozzle and blown up to the desired size as shown in Figure 4. During the inflation it is found that the liquid accelerator is caused by the stretching of the gel material to be absorbed into the gel. The gel is then dried in inflated condition as shown in Figure 4 and, when it has been dried, is deflated and heated in dry air at 212° F. to bring about vulcanization as shown in Figure 5. It is found that the vulcanization proceeds normally because of the presence of the accelerator which has been drawn into the gel during inflation.

It is essential that the step of soaking the gel article in the accelerator be carried out before the article is inflated, because, in addition to absorption of accelerator into the gel during soaking, there is a relatively enormous absorption of accelerator into the gel as the gel is expanded during inflation. By inflating the latex article while wet with an accelerator solution much more uniform and thorough association of the accelerator is achieved. The article will be found to have very uniform characteristics when vulcanized. This distinguishes the result sharply from prior procedures where the degree of vulcanization varies from place to place in accordance with the penetration of the accelerator into the gel and this in many instances is quite variable.

If it is desired, the accelerator may be introduced into the gel after the gel has been stripped

from the mold, although we have found that the gels may be more conveniently handled and immersed while they are still on the molds.

It will be appreciated that the objects of the invention may be attained by including in the dipping bath only a small amount of accelerator, the particular amount depending upon plant conditions.

The present invention, it will be appreciated, is equally applicable to the manufacture of other objects than the meteorological balloons selected as the specific example for purposes of disclosure. The present process may be used in the manufacture of any rubber article which lends itself to production by the process of our copending application, Serial No. 510,442 (on which the present invention is an improvement).

We claim:

1. The process of manufacturing rubber articles which comprises dipping a coagulant-coated mold into a liquid dispersion of natural rubber compounded for vulcanization except that it is deficient in accelerator, withdrawing the mold from the dispersion with a deposit of rubber gel thereon, soaking the gel in a liquid containing an accelerator of vulcanization, expanding the gel while it is still plastic and thereafter drying and vulcanizing the gel.

2. The process of manufacturing rubber articles which comprises dipping a coagulant-coated mold into a liquid dispersion of natural rubber compounded for vulcanization except that it is deficient in accelerator, withdrawing the mold from the dispersion with a deposit of rubber gel thereon, immersing the mold and gel in a liquid containing an accelerator of vulcanization, stripping the gel from the mold, expanding the gel while it is still plastic and thereafter drying and vulcanizing the gel.

3. The process of manufacturing rubber articles which comprises dipping a coagulant-coated mold into a liquid dispersion of natural rubber compounded for vulcanization except that it is deficient in accelerator, withdrawing the mold from the dispersion with a deposit of rubber gel thereon, stripping the gel from the mold, soaking the gel in a liquid containing an accelerator of vulcanization, expanding the gel while it is still plastic, and thereafter drying and vulcanizing the gel.

EMILE E. HABIB.  
GORDON E. GOTTE.